

## UNITED STATES PATENT OFFICE.

LOUIS D. SIMPKINS, OF BROOKLYN, NEW YORK, ASSIGNOR TO NATIONAL LEAD COMPANY, OF NEW YORK, N. Y., A CORPORATION OF NEW JERSEY.

## ELECTRODEPOSITION OF TIN.

No Drawing.

Application filed February 10, 1922. Serial No. 535,591.

*To all whom it may concern:*

Be it known that I, LOUIS D. SIMPKINS, a citizen of the United States, residing in Brooklyn, New York, U. S. A., have invented the following described Improvements in the Electrodeposition of Tin.

The object of this invention is to improve the process of electrolytic deposition of tin as for example in tin refining or tin-plating and consists in the composition of the bath and more particularly in the combination of a certain addition agent for use with the tin-salt solution to constitute the bath. According to this invention the salt solution is preferably stannous sulphate although other salts may be used, and the addition agent consists of beta-naphthol and a suitable colloid which are added to the salt solution in small amounts successively or as a mixture. And in general, as is well known in the art, the addition agent is added in amounts ranging from .01% to 2% by weight of the electrolyte, which proportions may be regarded as the minimum and maximum in this particular instance, although the range of greatest effectiveness is from .03% to .75% by weight of the electrolyte. The stannous sulphate solution may be conveniently prepared by electrolytically dissolving tin in sulphuric acid by the aid of a porous cell as well understood in this art and so as to leave some excess of free acid, in the solution, say about 10%. The beta-naphthol is added in the proportion of about one gram per litre of the electrolyte, and in order to render it miscible therewith it is dissolved in a small quantity of ethyl alcohol and introduced as a solution. The colloid is added in about the proportion of two grams to the litre being first dissolved in water to make about a 10% solution. The addition agent thus comprises beta-naphthol and a colloid in the proportions of one to two and as above stated they may be added, mixed together, or successively. While hide glue and other like substances may be usefully employed as the colloidal component, it is found that one of the peptones such for example as the common pharmaceutical peptone, which is quite soluble in water, forms the most elective combination with the beta-naphthol and the use of this particular

colloid in such combination is the preferred form of this invention. 55

The effect of this composite addition agent in the bath, is manifested by the deposit on the cathode of a compact, homogeneously dense and coherent layer of metallic tin which when used for tin-plating forms an adherent coating naturally so bright as to require very little subsequent polishing, and when used for refining tin, forms a plate of similar qualities which can be stripped from the cathode and 60 worked or melted practically without waste, and which is produced with relatively low consumption of current and hence at low cost. Other ingredients may also be present in the bath and in so far as they do not 65 destroy the effect of the beta-naphthol and the colloid, are included in this invention. I am aware that peptone has been heretofore suggested or employed as an addition agent in electrolytic tin-salt solutions and 70 also that beta-naphthol has been suggested as an addition agent for certain other salt solutions but I believe myself to have been the first to discover the particular utility 75 of the combination of beta-naphthol and peptone or equivalent colloid, in a tin-salt solution as a means of obtaining the results above referred to and this patent is 80 intended to cover that discovery without limitation except as specified in the following. 85

## Claims:

1. An electrolytic bath for depositing tin, containing a tin-salt solution and small amounts of beta-naphthol and a colloid. 90
2. An electrolytic bath for depositing tin, containing a tin-salt solution with free acid and small quantities of beta-naphthol and a colloid. 95
3. An electrolytic bath for depositing tin, containing stannous sulphate and small quantities of beta-naphthol and a colloid. 100
4. An electrolytic bath for depositing tin, comprising stannous sulphate with free sulphuric acid and small amounts of beta-naphthol and a colloid. 105
5. An electrolytic bath for depositing tin, comprising a tin-salt solution to which have been added small quantities of beta-naphthol and a colloid, in substantially the proportions of one to two.

6. An electrolytic bath for depositing tin, comprising a tin-salt solution and small amounts of beta-naphthol and peptone.
7. An electrolytic bath for the deposition of tin, containing stannous sulphate, and small amounts of beta-naphthol and a peptone.
8. An electrolytic bath for depositing tin, comprising stannous sulphate, free sulphuric acid and small amounts of beta-naphthol and a peptone.

In testimony whereof, I have signed this specification.

LOUIS D. SIMPKINS.